



US011545276B2

(12) **United States Patent**  
**Sommer et al.**

(10) **Patent No.:** **US 11,545,276 B2**  
(45) **Date of Patent:** **Jan. 3, 2023**

(54) **BORON X-RAY WINDOW**

(71) Applicant: **Moxtek, Inc.**, Orem, UT (US)

(72) Inventors: **Jared Sommer**, Bountiful, UT (US);  
**Jonathan Abbott**, Saratoga Springs, UT  
(US)

(73) Assignee: **Moxtek, Inc.**, Orem, UT (US)

(\*) Notice: Subject to any disclaimer, the term of this patent is extended or adjusted under 35 U.S.C. 154(b) by 158 days.

(21) Appl. No.: **17/228,846**

(22) Filed: **Apr. 13, 2021**

(65) **Prior Publication Data**

US 2021/0358652 A1 Nov. 18, 2021

**Related U.S. Application Data**

(60) Provisional application No. 63/023,385, filed on May 12, 2020.

(51) **Int. Cl.**

**H01J 35/18** (2006.01)  
**G21K 1/10** (2006.01)

(52) **U.S. Cl.**

CPC ..... **G21K 1/10** (2013.01)

(58) **Field of Classification Search**

CPC . A61B 6/032; H01J 35/16; H01J 35/18; H01J

2235/183; H01J 2231/50036; H01J 2235/1216; H01J 2235/18; H01J 2209/18; H01J 14/004; H01J 2235/122; H01J 35/32

See application file for complete search history.

(56) **References Cited**

**U.S. PATENT DOCUMENTS**

|                  |         |                        |
|------------------|---------|------------------------|
| 4,862,490 A      | 8/1989  | Karnezos et al.        |
| 10,636,614 B2    | 4/2020  | Sommer et al.          |
| 2008/0296479 A1  | 12/2008 | Anderson et al.        |
| 2009/0173897 A1  | 7/2009  | Decker et al.          |
| 2013/0051535 A1  | 2/2013  | Davis et al.           |
| 2017/0040138 A1  | 2/2017  | Kumar et al.           |
| 2018/0323033 A1  | 11/2018 | Black et al.           |
| 2019/0002298 A1  | 1/2019  | Hersam et al.          |
| 2019/0056654 A1  | 2/2019  | Peter et al.           |
| 2019/0214217 A1* | 7/2019  | Sommer ..... H01J 5/18 |

\* cited by examiner

*Primary Examiner* — Don K Wong

(74) *Attorney, Agent, or Firm* — Thorpe, North & Western, LLP

(57) **ABSTRACT**

An x-ray window can include a boron-film 12 and an aluminum-film 52 spanning an aperture 15 of a support-frame 11. The boron-film 12 and the aluminum-film 52 can be the only films, or the primary films, spanning the aperture. The boron-film 12 can include boron and hydrogen. An annular-film 32 can adjoin the support-frame 11, on an opposite side of the support-frame 11 from the boron-film 12. The annular-film 32 can include boron and hydrogen. The annular-film 32 can have the same material composition as, and can be similar in thickness with, the boron-film 12.

**20 Claims, 4 Drawing Sheets**



*Fig. 1*



*Fig. 2*



*Fig. 3*



*Fig. 4*



*Fig. 5*



*Fig. 6*



*Fig. 7*



*Fig. 8*



*Fig. 9*

**1**  
**BORON X-RAY WINDOW**

CLAIM OF PRIORITY

This application claims priority to U.S. Provisional Patent Application No. 63/023,385, filed on May 12, 2020, which is incorporated herein by reference.

FIELD OF THE INVENTION

The present application is related to x-ray windows.

BACKGROUND

X-ray windows are used in expensive systems requiring high reliability. High system requirements result in demanding characteristics of the x-ray window.

BRIEF DESCRIPTION OF THE DRAWINGS  
(DRAWINGS MIGHT NOT BE DRAWN TO SCALE)

FIG. 1 is a cross-sectional side-view of an x-ray window 10 comprising a boron-film 12 hermetically sealed to a support-frame 11, the support-frame 11 encircling an aperture 15.

FIG. 2 is a bottom-view (support-frame 11 side) of the x-ray window 10 of FIG. 1.

FIG. 3 is a cross-sectional side-view of an x-ray window 30 comprising a support-frame 11 encircling an aperture 15 and having a top-side 11<sub>T</sub> and a bottom-side 11<sub>B</sub>, a boron-film 12 on the top-side 11<sub>T</sub> of the support-frame 11, and an annular-film 32 on the bottom-side 11<sub>B</sub> of the support-frame 11.

FIG. 4 is a schematic bottom-view (annular-film 32 side) of the x-ray window 30 of FIG. 3.

FIG. 5 is a cross-sectional side-view of an x-ray window 50, similar to x-ray windows 10 and 30, but further comprising a thin film 52 on a far-side 12<sub>F</sub> of the boron-film 12, further from the support-frame 11.

FIG. 6 is a cross-sectional side-view of an x-ray window 60, similar to x-ray window 10, but further comprising a thin film 52 on a near-side 12<sub>N</sub> of the boron-film 12, nearer to the support-frame 11.

FIG. 7 is a cross-sectional side-view of an x-ray window 70, similar to x-ray window 30, but further comprising a thin film 52 on a near-side 12<sub>N</sub> of the boron-film 12, nearer to the support-frame 11.

FIG. 8 is a cross-sectional side-view illustrating step 80 in a method of making an x-ray window, including placing a wafer 81 in an oven, and forming a boron-film 12 on the wafer.

FIG. 9 is a cross-sectional side-view illustrating step 90 in a method of making an x-ray window, including: placing a wafer 81 in an oven, the wafer 81 having a top-side 81<sub>T</sub> and a bottom-side 81<sub>B</sub>; and forming an upper-boron-film 12<sub>u</sub> on the top-side 81<sub>T</sub> of the wafer 81 and a lower-boron-film 12<sub>L</sub> on the bottom-side 81<sub>B</sub> of the wafer 81.

DEFINITIONS

The following definitions, including plurals of the same, apply throughout this patent application.

As used herein, the term "identical material composition" means exactly identical or identical within normal manufacturing tolerances.

**2**

As used herein, the term "g/cm<sup>3</sup>" means grams per cubic centimeters.

As used herein, the term "minimum thickness" means the smallest/minimum thickness of the specified material in the aperture 15 or 35.

As used herein, the terms "on", "located at", and "adjacent" mean located directly on or located over with some other solid material between. The terms "located directly on", "adjoin", "adjoins", and "adjoining" mean direct and immediate contact.

As used herein, the term "nm" means nanometer(s).

As used herein, the term "parallel" means exactly parallel, parallel within normal manufacturing tolerances, or nearly parallel such that any deviation from exactly parallel would have negligible effect for ordinary use of the device.

As used herein, the terms "top-side" and "bottom-side" refer to top and bottom-sides or faces in the figures, but the device may be oriented in other directions in actual practice.

20 The terms "top" and "bottom" are used for convenience of referring to these sides or faces.

REFERENCE NUMBERS IN THE DRAWINGS

10, 30, 50, 60, and 70 are x-ray window embodiments.

The support-frame 11 can encircle an aperture 15. The support-frame 11 can include an inner-side 11<sub>i</sub> facing the aperture 15 and an outer-side 11<sub>o</sub> facing outward and opposite of the inner-side 11<sub>i</sub>. The support-frame 11 can include a top-side 11<sub>T</sub> and a bottom-side 11<sub>B</sub> opposite of each other.

The boron-film 12 can include a near-side 12<sub>N</sub> (nearer the support-frame 11) and a far-side 12<sub>F</sub> (farther from the support-frame 11). Method step 90 shows an upper-boron-film 12<sub>u</sub> and a lower-boron-film 12<sub>L</sub>.

35 The annular-film 32 can include an aperture 35, a near-side 32<sub>N</sub> (nearer the support-frame 11) and a far-side 32<sub>F</sub> (farther from the support-frame 11).

The thin-film 52 can be an aluminum-film or a film made of another material. The thin-film 52 can be a stack of 40 multiple layers/multiple thin-films.

80 and 90 are steps in a method of making x-ray windows. Wafer 81 has a top-side 81<sub>T</sub> and a bottom-side 81<sub>B</sub>. Wafer 81 is located in an oven 82.

DETAILED DESCRIPTION

Useful characteristics of x-ray windows include low gas permeability, low outgassing, high strength, low visible and infrared light transmission, high x-ray flux, made of low atomic number materials, corrosion resistance, high reliability, and low-cost. Each x-ray window design is a balance between these characteristics.

An x-ray window can combine with a housing to enclose an internal vacuum. The internal vacuum can aid device 55 performance. For example, an internal vacuum for an x-ray detector (a) minimizes gas attenuation of incoming x-rays and (b) allows easier cooling of the x-ray detector.

Permeation of a gas through the x-ray window can degrade the internal vacuum. Thus, low gas permeability is 60 a desirable x-ray window characteristic.

Outgassing from x-ray window materials can degrade the internal vacuum of the device. Thus, selection of materials with low outgassing is useful.

The x-ray window can face vacuum on one side and atmospheric pressure on an opposite side. Therefore, the x-ray window may need strength to withstand this differential pressure.

Visible and infrared light can cause undesirable noise in the x-ray detector. The ability to block transmission of visible and infrared light is another useful characteristic of x-ray windows.

A high x-ray flux through the x-ray window allows rapid functioning of the x-ray detector. Therefore, high x-ray transmissivity through the x-ray window is useful.

Detection and analysis of low-energy x-rays is needed in some applications. High transmission of low-energy x-rays is thus another useful characteristic of x-ray windows.

X-rays can be used to analyze a sample. X-ray noise from surrounding devices, including from the x-ray window, can interfere with a signal from the sample. X-ray noise from high atomic number materials are more problematic. It is helpful, therefore, for the x-ray window to be made of low atomic number materials.

X-ray windows are used in corrosive environments, and may be exposed to corrosive chemicals during manufacturing. Thus, corrosion resistance is another useful characteristic of an x-ray window.

X-ray window failure is intolerable in many applications. For example, x-ray windows are used in analysis equipment on Mars. High reliability is a useful x-ray window characteristic.

X-ray window customers demand low-cost x-ray windows with the above characteristics. Reducing x-ray window cost is another consideration.

The present invention is directed to various x-ray windows, and methods of making x-ray windows, that satisfy these needs. Each x-ray window or method may satisfy one, some, or all of these needs.

As illustrated in FIGS. 1-7, x-ray windows 10, 30, 50, 60, and 70 can include a boron-film 12 on a support-frame 11, and spanning an aperture 15 of the support-frame 11. These x-ray windows 10, 30, 50, 60, and 70 can include the following characteristics: low gas permeability, low outgassing, high strength, low visible and infrared light transmission, high x-ray flux, made of low atomic number materials, corrosion resistance, high reliability, and low-cost.

The boron-film 12 can be the main support structure spanning the aperture 15 of the support-frame 11, and can be thicker than any other material spanning the aperture 15. Example lower limits of a minimum thickness  $Th_{12}$  of the boron-film 12 across the aperture include:  $Th_{12} \geq 25$  nm,  $Th_{12} \geq 50$  nm,  $Th_{12} \geq 100$  nm,  $Th_{12} \geq 300$  nm, or  $Th_{12} \geq 500$  nm. Example upper limits of a minimum thickness  $Th_{12}$  of the boron-film 12 across the aperture include: and  $Th_{12} \leq 500$  nm,  $Th_{12} \leq 750$  nm,  $Th_{12} \leq 1200$  nm,  $Th_{12} \leq 1500$  nm,  $Th_{12} \leq 3000$  nm, or  $Th_{12} \leq 10,000$  nm.

The support-frame 11 can have a ring shape, can encircle the aperture 15, or both. The support-frame 11 can have a top-side 11<sub>T</sub> and a bottom-side 11<sub>B</sub>, which can be opposite of each other and parallel with respect to each other. The support-frame 11 can have an inner-side 11<sub>i</sub> facing the aperture 15 and an outer-side 11<sub>o</sub> opposite of the inner-side 11<sub>i</sub>. The inner-side 11<sub>i</sub> and the outer-side 11<sub>o</sub> can extend between and can join the top-side 11<sub>T</sub> and the bottom-side 11<sub>B</sub>. The support-frame 11 (and the wafer 81 described below) can comprise silicon, such as for example  $\geq 30$ ,  $\geq 50$ ,  $\geq 90$ , or  $\geq 95$  mass percent silicon. The support-frame 11 (and the wafer 81 described below) can comprise silicon dioxide, such as for example  $\geq 30$ ,  $\geq 50$ ,  $\geq 90$ , or  $\geq 95$  mass percent silicon dioxide.

The boron-film 12 can have a near-side 12<sub>N</sub> (nearer the support-frame 11) and a far-side 12<sub>F</sub> (farther from the support-frame 11), opposite of each other. The near-side 12<sub>N</sub> of the boron-film 12 can adjoin and/or be hermetically-

sealed to the top-side 11<sub>T</sub> of the support-frame 11. The hermetic-seal can be a direct bond between the top-side 11<sub>T</sub> of the support-frame 11 and the boron-film 12. The hermetic-seal can be free of aluminum or an aluminum-film.

Example weight percentages of boron, throughout the entire boron-film 12, include  $\geq 80$ ,  $\geq 90$ ,  $\geq 95$ ,  $\geq 97$ ,  $\geq 98$ , or  $\geq 99$  weight percent. Example weight percentages of hydrogen, throughout the entire boron-film 12, include  $\geq 0.01$ ,  $\geq 0.05$ ,  $\geq 0.1$ ,  $\geq 0.5$ ,  $\geq 0.9$ ,  $\geq 2$ , or  $\geq 4$  weight percent hydrogen.

Example density, throughout the entire boron-film 12, includes  $\geq 1.94$  g/cm<sup>3</sup>,  $\geq 2.04$  g/cm<sup>3</sup>, or  $\geq 2.1$  g/cm<sup>3</sup> and  $\leq 2.18$  g/cm<sup>3</sup>,  $\leq 2.24$  g/cm<sup>3</sup>, or  $\leq 2.34$  g/cm<sup>3</sup>. For example, the boron-film 12 can have 99.1 weight percent boron, 0.9 weight percent hydrogen, and density of 2.14 g/cm<sup>3</sup>. A window with these material properties can be manufactured as noted in the METHOD section below.

The aperture 15 of the support-frame 11 can consist of thin films spanning the entire aperture. The aperture 15 of the support-frame 11 can be free of material of the support-frame 11, free of ribs, or both.

As illustrated in FIGS. 3-4 and 7, x-ray windows 30 and 70 can further comprise an annular-film 32 on the bottom-side 11<sub>B</sub> of the support-frame 11. The annular-film 32 can be hermetically-sealed to the support-frame 11. The annular-film 32 can adjoin the bottom-side 11<sub>B</sub> of the support-frame 11. An aperture 35 of the annular-film 32 can be aligned with the aperture 15 of the support-frame 11. The annular-film 32 can be absent from, not extend into, and not cross the aperture 15 of the support-frame 11. The annular-film 32 can have material composition as described above for the boron-film 12. The boron-film 12 and the annular-film 32 can have an identical material composition. The boron-film 12 and the annular-film 32 can have similar thickness. For example 35  $|Th_{12} - Th_{32}|/Th_{12}$ , where  $Th_{12}$  is a minimum thickness of the boron-film 12 and  $Th_{32}$  is a minimum thickness of the annular-film 32.

Addition of the annular-film 32 can improve the ability of the x-ray window to withstand thermal stress during rapid or large temperature changes and can improve bonding of the x-ray window to a housing. The above benefits are particularly applicable if the annular-film 32 is similar in material and thickness to the boron-film 12.

X-ray windows 30 and 70, with the annular-film 32, can be combined with any other x-ray window examples described herein, including those shown in any of FIGS. 1 and 5-6.

As illustrated in FIGS. 5-7, a stack of films, including the boron-film 12 and a thin-film 52, can span the aperture 15 of the support-frame 11. The thin-film 52 can be an aluminum-film. Example material compositions of the aluminum-film include  $\geq 25$ ,  $\geq 50$ , or  $\geq 75$  weight percent aluminum throughout the entire aluminum-film. Addition of the aluminum-film can improve the ability of the x-ray window to block visible light. The aperture 15 can consist only of the boron-film 12 and the aluminum-film.

The thin-film 52 can be located on the far-side 12<sub>F</sub> of the boron-film 12, as illustrated in FIG. 5. Because of superior corrosion resistance of the boron-film 12, a more likely location for the thin-film 52 is on the near-side 12<sub>N</sub>, as illustrated in FIGS. 6-7. The thin-film 52 can adjoin a central portion of the near-side 12<sub>N</sub> of the boron-film 12.

The thin-film 52 on the far-side 12<sub>F</sub> of the boron-film 12 can be combined with the annular-film 32 (FIGS. 3 and 7). The thin-film 52 on the far-side 12<sub>F</sub> of the boron-film 12 can be combined with the thin-film 52 on the near-side 12<sub>N</sub> (FIGS. 6-7).

An outer portion or outer ring of the near-side  $12_N$  of the boron-film  $12$  can be attached to or adjoin the support-frame  $11$ . A junction of the boron-film  $12$  and the support-frame  $11$  can be free of the thin-film  $52$ .

The thin-film  $52$  can extend onto, cover, or adjoin the inner-side  $11_i$  and the bottom-side  $11_B$  of the support-frame  $11$ , as illustrated in FIG. 6. The thin-film  $52$  can extend onto, cover, or adjoin the inner-side  $11_i$  of the support-frame  $11$  and the far-side  $32_F$  of the annular-film  $32$ , as illustrated in FIG. 7.

Because aluminum has a higher atomic number than boron, it can be useful to have a relatively thin layer of aluminum. Thus for example,  $Th_{52} \leq 0.5 * Th_{12}$ ,  $Th_{52} \leq 0.3 * Th_{12}$ ,  $Th_{52} \leq 0.1 * Th_{12}$ , where  $Th_{52}$  is a minimum thickness of the thin-film  $52$  in the aperture  $15$  and  $Th_{12}$  is a minimum thickness of the boron-film  $12$  in the aperture  $15$ . Other example relationships, for the thin-film  $52$  to have sufficient thickness, include  $Th_{52} \geq 0.001 * Th_{12}$ ,  $Th_{52} \geq 0.01 * Th_{12}$ , or  $Th_{52} \geq 0.1 * Th_{12}$ .

The boron film  $12$  can be the primary film or only film spanning the aperture  $15$ . Thus, for example,  $Th_F \leq 1.1 * Th_{12}$ ,  $Th_F \leq 1.25 * Th_{12}$ ,  $Th_F \leq 1.5 * Th_{12}$ , or  $Th_F \leq 2 * Th_{12}$ .

The aluminum-film and the boron-film  $12$  can be the only solid structures spanning the aperture  $15$  of the support-frame  $11$ . The boron film  $12$  and the aluminum-film can be the primary films, or only films, spanning the aperture  $15$ . Thus, for example,  $Th_F \leq 1.1 * (Th_{12} + Th_{52})$ ,  $Th_F \leq 1.25 * (Th_{12} + Th_{52})$ ,  $Th_F \leq 1.5 * (Th_{12} + Th_{52})$ , or  $Th_F \leq 2 * (Th_{12} + Th_{52})$ .  $Th_F$  is a minimum thickness of the films in the aperture  $15$ .

The x-ray window can be hermetically sealed to a housing, with an internal vacuum. The boron-film  $12$  can face atmospheric pressure and the aluminum-film can face a vacuum.

#### Method

A method of manufacturing an x-ray window can comprise some or all of the following steps, which can be performed in the following order. There may be additional steps not described below. These additional steps may be before, between, or after those described.

The method can comprise placing a wafer  $81$  in an oven  $82$ ; introducing a gas into the oven  $82$ , the gas including boron, and forming boron-film(s)  $12$  on the wafer  $81$  (step 30 in FIG. 8 or step 90 in FIG. 9). The gas can include diborane, such as for example  $\geq 5$  molar percent diborane and  $\geq 70$  molar percent argon.

Deposition temperature can be adjusted to control percent hydrogen and percent boron. Lower (higher) temperature can result in increased (decreased) hydrogen in the boron-film  $12$ . For example, a temperature of  $390^\circ C$ . can result in about 1% H in the boron-film  $12$ . Other example temperatures in the oven  $82$ , during formation of the boron-film(s)  $12$ , include  $\geq 50^\circ C$ .,  $\geq 100^\circ C$ .,  $\geq 200^\circ C$ .,  $\geq 300^\circ C$ ., or  $\geq 340^\circ C$ ., and  $\leq 340^\circ C$ .,  $\leq 380^\circ C$ .,  $\leq 450^\circ C$ .,  $\leq 525^\circ C$ .,  $\leq 550^\circ C$ ., or  $\leq 600^\circ C$ .

Formation of the boron-film  $12$  can be plasma enhanced, in which case the temperature of the oven  $82$  can be relatively lower. A pressure in the oven can be relatively low, such as for example 60 pascal. Higher pressure deposition might require a higher process temperature.

As illustrated in FIG. 9, the wafer  $81$  can have a top-side  $81_T$  and a bottom-side  $81_B$ . The top-side  $81_T$  and the bottom-side  $81_B$  can be opposite of each other and can be parallel with respect to each other. Both the top-side SIT and the bottom-side  $81_B$  can be exposed to the gas (mount or hold the wafer at its outer edges). Forming the boron-film(s)  $12$  can include forming an upper-boron-film  $12_U$  on the top-side

$81_T$  of the wafer  $81$  and forming a lower-boron-film  $12_L$  on the bottom-side  $81_B$  of the wafer  $81$ .

Here is an example of deposition to form boron-film(s)  $12$  with about 99.1 weight percent boron, 0.9 weight percent hydrogen, and density of  $2.14 \text{ g/cm}^3$ . A wafer  $81$  is loaded into the oven  $82$ . The furnace is evacuated (about 450 mTorr) and temperature stabilized at  $\sim 390^\circ C$ . A gas with 15 molar percent diborane and 85 molar percent argon is introduced into the oven, resulting in deposition of the 10 boron-film(s)  $12$ . Oven  $82$  pressure is controlled by an adjustable butterfly valve at the vacuum inlet.

After step 80, the method can further comprise etching through a center of the wafer  $81$  at the bottom-side  $81_B$  to form a support-frame  $11$  encircling an aperture  $15$  (see FIGS. 1-2).

After step 90, the method can further comprise etching through a center of the lower-boron-film  $12_S$  to form an annular-film  $32$  and etching through a center of the wafer  $81$  at the bottom-side  $81_B$  to form a support-frame  $11$  encircling an aperture  $15$  (see FIGS. 3-4). The annular-film  $32$  can be used as a mask to etch the wafer  $81$  to form the support-frame  $11$ . Etch of the wafer can continue up to the boron-film  $12$  or upper-boron-film  $12_U$ .

A resist can be used to form the desired annular-shape of the annular-film  $32$  or the support-frame  $11$ . A solution of potassium ferricyanide, a fluorine plasma (e.g. NF<sub>3</sub>, SF<sub>6</sub>, CF<sub>4</sub>), or both, can be used to etch the lower-boron-film  $12_S$ . Example chemicals for etching the wafer  $81$  include ammonium hydroxide, cesium hydroxide, potassium ferricyanide, potassium hydroxide, sodium hydroxide, sodium oxalate, tetramethylammonium hydroxide, or combinations thereof. The resist can then be stripped, such as for example with sulfuric acid and hydrogen peroxide (e.g. Nanostrip).

Some (e.g.  $\geq 25\%$ ,  $\geq 50\%$ ,  $\geq 75\%$ , or  $\geq 90\%$ ) of the near-side  $12_N$  and the far-side  $12_F$  of the boron-film  $12$  can both face atmospheric pressure, a gas, or both at this step in the process (after etch and before the deposition of thin-film 35  $52$ /aluminum-film).

A thin-film  $52$  (e.g. an aluminum-film) can be deposited 40 on the far-side  $12_F$  of the boron-film  $12$  (FIG. 5).

A thin-film  $52$  (e.g. an aluminum-film) can be deposited on the near-side  $12_N$  of the boron-film  $12$  (or the near-side  $12_N$  of the upper-boron-film  $12_U$ ), on the inner-side  $11_i$  of the support-frame  $11$ , on the bottom-side  $11_B$  of the support-frame  $11$ , or combinations thereof (FIG. 6). If the x-ray window includes the annular-film  $32$ , then deposition can occur on an inside surface and the far-side  $32_F$  of the annular-film  $32$  instead of on the bottom-side  $11_B$  of the support-frame  $11$  (FIG. 7). The method can further comprise applying an adhesion layer (e.g. Cr, Si, Zn) on the boron-film  $12$  before applying, or during application of, the aluminum-film.

The x-ray window can then be sealed to a housing with a vacuum inside of the housing. The boron-film  $12$  (or upper-boron-film  $12_U$ ) can face atmospheric pressure outside of the housing, and the aluminum-film can face the vacuum.

The support-frame  $11$ , boron-film(s)  $12$ , annular-film  $32$ , and the thin-film(s)  $52$  can have properties as described above.

What is claimed is:

1. An x-ray window comprising:  
a support-frame encircling an aperture and having a top-side and a bottom-side, the top-side and the bottom-side parallel with respect to each other;  
a boron-film and an aluminum-film spanning the aperture of the support-frame;

the boron-film having  $\geq 90$  weight percent boron throughout the entire boron-film, and having a near-side and a far-side opposite of each other; a hermetic-seal between and adjoining an outer-ring of the near-side of the boron-film and the top-side of the support-frame, the hermetic-seal is a direct bond between the boron-film and the support-frame and is free of the aluminum-film; the aluminum-film adjoins the near-side of the boron-film inside of the outer-ring;  $Th_F \leq 1.25 * (Th_{12} + Th_{52})$ , where  $Th_F$  is a minimum thickness of all thin films spanning the aperture,  $Th_{12}$  is a minimum thickness of the boron-film in the aperture, and  $Th_{52}$  is a minimum thickness of the aluminum-film in the aperture; and an annular-film adjoining the bottom-side of the support-frame, having an aperture aligned with the aperture of the support-frame, and including  $\geq 90$  weight percent boron throughout the entire annular-film.

2. The x-ray window of claim 1, wherein the aperture of the support-frame is free of support ribs and  $300 \text{ nm} \leq Th_{12} \leq 1200 \text{ nm}$ .

3. The x-ray window of claim 1, wherein the aperture of the support-frame is free of material of the support-frame.

4. The x-ray window of claim 1, wherein solid material in the aperture consists of thin films spanning the entire aperture.

5. The x-ray window of claim 1, wherein a maximum total thickness of all thin films in the aperture is  $\leq 4000 \text{ nm}$ .

6. The x-ray window of claim 1, wherein a percent thickness difference between the boron-film and the annular-film is  $\leq 20\%$ , where the percent thickness difference equals a difference in minimum thickness between the boron-film and the annular-film divided by a minimum thickness of the boron-film.

7. The x-ray window of claim 1, further comprising  $\geq 0.05$  weight percent hydrogen throughout the entire boron-film and the entire annular-film.

8. The x-ray window of claim 1, wherein the boron-film and the annular-film have an identical material composition.

9. An x-ray window comprising:  
a support-frame encircling an aperture and having a top-side and a bottom-side, the top-side and the bottom-side parallel with respect to each other;  
a boron-film hermetically-sealed to the top-side, spanning the aperture of the support-frame, the boron-film having  $\geq 90$  weight percent boron throughout the entire boron-film; and  
an annular-film hermetically-sealed to the bottom-side, having an aperture aligned with the aperture of the support-frame, and including  $\geq 90$  weight percent boron throughout the entire annular-film.

10. The x-ray window of claim 9, wherein  $Th_F \leq 1.5 * Th_{12}$ , where  $Th_F$  is a minimum thickness of all thin films spanning the aperture, and  $Th_{12}$  is a minimum thickness of the boron-film in the aperture.

11. The x-ray window of claim 9, further comprising an aluminum-film spanning the aperture of the support-frame; the aluminum-film having  $\geq 50$  weight percent aluminum throughout the entire aluminum-film; and the aluminum-film and the boron-film are the only solid structures spanning the aperture of the support-frame.

12. The x-ray window of claim 9, further comprising an aluminum-film spanning the aperture of the support-frame, the boron-film faces atmospheric pressure, and the aluminum-film faces a vacuum.

13. The x-ray window of claim 9, wherein a percent thickness difference between the boron-film and the annular-film is  $\leq 20\%$ , where the percent thickness difference equals a difference in minimum thickness between the boron-film and the annular-film divided by a minimum thickness of the boron-film.

14. The x-ray window of claim 9, further comprising  $\geq 0.05$  weight percent hydrogen throughout the entire boron-film and the entire annular-film.

15. The x-ray window of claim 9, wherein the boron-film and the annular-film have an identical material composition.

16. An x-ray window comprising:  
a support-frame encircling an aperture;  
a boron-film spanning the aperture and hermetically-sealed to the support-frame;  
the boron-film having  $\geq 97$  weight percent boron,  $\geq 0.3$  weight percent hydrogen, and a density of  $\geq 2.04 \text{ g/cm}^3$  and  $\leq 2.24 \text{ g/cm}^3$ ;

$Th_F \leq 1.5 * Th_{12}$ , where  $Th_F$  is a minimum thickness of all solid structures spanning the aperture and  $Th_{12}$  is a minimum thickness of the boron-film in the aperture.

17. The x-ray window of claim 16, further comprising:  
the support-frame has a top-side and a bottom-side opposite of each other;  
the boron-film is hermetically-sealed to the top-side; and  
an annular-film hermetically-sealed to the bottom-side, having  $\geq 97$  weight percent boron,  $\geq 0.3$  weight percent hydrogen, and a density of  $\geq 2.04 \text{ g/cm}^3$  and  $\leq 2.24 \text{ g/cm}^3$ .

18. The x-ray window of claim 16, further comprising an aluminum-film adjoining an inner-side and a bottom-side of the support-frame.

19. The x-ray window of claim 17, wherein the boron-film faces atmospheric pressure and the aluminum-film faces a vacuum.

20. The x-ray window of claim 16, wherein the aperture is free of support ribs and  $300 \text{ nm} \leq Th_{12} \leq 1200 \text{ nm}$ .

\* \* \* \* \*